

1

3,459,662

## PHOSPHO-SULFURIZED PHOSPHITE ESTERS AND HYDROCARBON COMPOSITIONS CONTAINING THE SAME

Shih-En Hu, Roselle, N.J., assignor to Esso Research and Engineering Company, a corporation of Delaware  
No Drawing. Filed Jan. 31, 1967, Ser. No. 612,794  
Int. Cl. C10m 5/24, 7/46; C07f 9/04

U.S. Cl. 252—46.7

11 Claims

## ABSTRACT OF THE DISCLOSURE

Reaction products of organic phosphite esters (mono-, di-, or tri-) with a phosphorus polysulfide are sludge inhibitors and anti-wear agents in lubricating oils or in middle distillate hydrocarbon fuels or residual hydrocarbon fuels, when used in amounts up to 10 wt. percent based on the weight of the compounded compositions.

The present invention relates to the production of phosphite ester reaction products with phosphorus polysulfides, which products are found to be particularly useful as additives when employed, in minor amounts, in hydrocarbon lubricating oils, in middle distillate hydrocarbon fuels, or in residual hydrocarbon fuels. Such reaction products have been found to be particularly useful as additives in these hydrocarbon compositions in order to inhibit oxidation, rust formation, sludge production, wear, and for dispersing any sludge which is formed and to the extent it is formed; thus preventing its deposit on the surfaces of automotive engines, fuel pumps, and the like where it would cause fouling and plugging difficulties.

Various phosphite derivatives have, in the past, been produced and used as additives in both hydrocarbon fuel compositions and in lubricating oil compositions for the purpose of inhibiting the corrosion of bearings, minimizing bearing wear, and for the purpose of otherwise protecting the internal metal surfaces of pumps and automotive engines. This is accomplished by imparting load carrying ability to the lubricating oils, limiting the corrosion of bearings in engines and pumps, and improving the wear qualities of the bearings and pumps and in internal combustion engines. The problem of rust is minimized in fuel pumps handling residual or middle distillate hydrocarbon fractions and fuels. Many of these phosphite compounds have exhibited one or more of the aforementioned characteristics but few, if any, have been found to satisfactorily cope with all or a majority of these problems from a commercial standpoint. High operating temperatures in internal combustion engines tend to assert accelerated detrimental oxidative influences on lubricating oils and this, of course, tends to result in the premature breakdown of these oils with the resultant formation of acids and other sludge-type materials which generally gum up, clog, and corrode bearings and internal surfaces leading to excessive wear of bearing surfaces and plugging difficulties in oil circulation systems because of the excessive quantities of sludge formed. It is recognized that sludge formation, whether or not the sludge is deposited, is an undesirable phenomenon associated with the use of lubricating oils and is to be minimized or avoided altogether if it is possible to do so.

The hereinafter, more fully described novel phosphite additives are ashless in nature which means that they tend to eliminate the formation of deposits in combustion chambers and in the crankcases of internal combustion engines where metal-containing sludge dispersants would, in fact, leave a residue or ash-forming deposits under like circumstances. Many of the heretofore prepared metallic dispersants have certain disadvantages. Some of

2

them are, for example, too corrosive to be used in lubricants or, because they have been neutralized with calcium carbonate or sodium hydroxide, they contain metallic constituents which form ash. They may also be too corrosive, for practical purposes, toward copper-lead bearings or silver-cadmium bearings. They may not, in themselves, exhibit antioxidant properties and antiwear properties in the oils containing them thus making it necessary to add other compounds to take care of these problems arising by reason of the high temperature operation of internal combustion engines. The novel phospho-sulfurized phosphite products hereinafter described accomplish the desired ends to a greater extent than has heretofore been thought to be possible or attainable.

The novel phospho-sulfurized phosphite esters which serve as additives for middle distillate fuels, residual hydrocarbon fuels and as additives in lubricating oils are prepared by reacting a mono-, di-, or tri- organic phosphite ester with a polysulfide of phosphorus in liquid phase and at elevated or superatmospheric temperatures for a sufficient length of time to introduce a polysulfide of phosphorus into the phosphite ester. The reactant organic phosphite ester may be represented by the formula:



wherein: R is a hydrocarbon radical selected from the group consisting of alkyl, chloralkyl, aryl, chloraryl, alkaryl, chloralkaryl, cyclo alkyl, chlorocyclo alkyl, alkenyl, chloralkenyl, aralkyl, and chloraralkyl; and R<sub>2</sub> and R<sub>3</sub> are hydrogen or the same as R<sub>1</sub>. These phospho-sulfurized esters have been found to exhibit outstanding antioxidant, antiwear and sludge inhibiting properties when employed in lubricating oils for internal combustion engines or in fuels. They are soluble in the above-mentioned hydrocarbon fuels and lubricating oils at least to the extent of about 10 wt. percent which is generally the upper limit of an amount suitable for use in either type of hydrocarbon mixture, i.e., lubricating oil or fuel. Further quantities or higher degrees of solubility are unnecessary because the additives do not perform their functions to any greater degree or with any better results than through the use of 10% or less of the additives. These novel additives are excellent in inhibiting the formation of sludge, in minimizing bearing weight loss and they exhibit outstanding qualities in being able to disperse and maintain in dispersion any small amounts of sludge that does form during the use of lubricating oils containing these novel sulfurized phosphite ester reaction product additives.

The phosphite esters employed as reactants may be either the monoester, the diester, or the triester of phosphorous acid or mixtures of two or more of these esters. Many of the esters employed in making useful additives, particularly those containing the smaller number of carbon atoms per molecule, are readily available commercially and their methods of preparation are conventional. Some of the esters, particularly those having the longer alkyl chains or hydrocarbon radicals or chlorinated hydrocarbon radicals of the higher number of carbon atoms per radical, although presently not available commercially, are readily prepared by the reacting of one, two, or three moles of the corresponding alcohol with one mole of phosphorous trihalide such as phosphorous trichloride or phosphorous tribromide. This is a conventional reaction and while there are other ways, also conventional, of producing these various phosphite esters, the present invention is not concerned with the particular method by which the phosphite esters are produced. In those cases where mono- or di-esters are formed, it is sometimes desirable, following the esterification reaction,

to treat the reacted mixture with water, dilute aqueous caustic, or dilute aqueous mineral acid in order to hydrolyze off the residual chlorine or bromine atoms present by reason of the trivalent phosphorous compound employed as the original reactant. Once this is accomplished, the mono-, di-, or tri-organic phosphite ester, or mixtures of two or more of these, may be readily phosphosulfurized with a phosphorous polysulfide but, surprisingly, it has been found that effective additives are not produced if the phosphorus sulfide is present in and during the phosphite esterification reaction. Only after the completion of the esterification reaction and the removal of reactant halogen is it possible to treat with phosphorus polysulfide and secure an effective antioxidant, sludge inhibiting, antiwear agent.

Any of the phosphorus polysulfides conveniently available, i.e., commercially marketed, may be employed. Representative of these specific compounds are the following:

P<sub>4</sub>S<sub>3</sub>—phosphorus sesquisulfide  
P<sub>3</sub>S<sub>6</sub>—phosphorus disulfide  
P<sub>4</sub>S<sub>6</sub>—phosphorus trisulfide  
P<sub>2</sub>S<sub>5</sub>—phosphorus pentasulfide

Specific phosphite esters which are useful as reactants with the polysulfides of phosphorus are exemplified by the following specific phosphites. (A specific listing of the mono ester is intended to include like listing of the diester and triester as well; thus, for example, methyl phosphite is intended to also include dimethyl phosphite and trimethyl phosphite.)

Methyl phosphite, ethyl phosphite, n-propyl phosphite, isopropyl phosphite, butyl phosphite, pentyl phosphite, hexyl phosphite, cyclohexyl phosphite, heptyl phosphite, nonyl phosphite, decyl phosphite, lauryl phosphite, lorol phosphite, cetyl phosphite, octadecyl phosphite, heptadecyl phosphite, phenyl phosphite, alpha or beta naphthyl phosphite, alpha or beta naphthenyl phosphite, benzyl phosphite, tolyl phosphite.

The mixed aryl phosphites, for example:

Methyl,phenyl phosphite; dimethyl,phenyl phosphite; amyl,phenyl phosphite; diamyl,phenyl phosphite; nonyl,phenyl phosphite, nonyl,phenyl phosphite; (4-amyl,phenyl) phosphite, 4-amylphenyl diethyl phosphite, di-octadecyl phenyl phosphite, octadecyl di-phenyl phosphite, isobutyl phenyl phosphite, nonyltolyl phosphite, nonyl,ditolyl phosphite; polyisobutyl diphenyl phosphite, di-polyisobutyl phosphite, di-polyisobutyl phenyl phosphite, (polyisobutyl phenyl) phosphite, chlorethyl phosphite, chlorbutyl phosphite, chloroctyl phosphite, chlor-phenyl phosphite, chlorbenzyl phosphite, chlorotolyl phosphite, (chloropolysobutyl diphenyl) phosphite, di-polyisobutyl (chlorbenzyl) phosphite, di-polyisobutyl (chlorpolysobutyl) phosphite.

The lorol radicals mentioned above in connection with the specific phosphites that may be employed are derived from the corresponding primary alcohols obtained by the carboxylic reduction of cocoanut or palm kernel oils. These crude mixtures contain a major amount of lorol alcohol together with minor amounts of octyldecyl and myristyl alcohols. A typical lorol mixture boils between about 140° C. and about 190° C. at 50 mm. mercury pressure.

The interaction of the heretofore mentioned phosphite esters with a phosphorus polysulfide is carried out in liquid phase either in the presence or absence of inert solvents such as normally liquid hydrocarbon petroleum solvents, for example, petroleum ether, hexane, chlorhexane, hexene, nonyl heptane, benzene, toluene, and the like. The reaction is generally carried out in the absence of solvents and between 1 and 3 moles of phosphite are employed per mole of phosphorus polysulfide; the sulfide being gradually and directly added to the phosphite, starting at ambient temperatures, for about 1 hour, after which the temperature may be gradually increased up to

5 between about 40° C. and about 200° C., preferably between about 75° C. and 120° C. The period of reaction, i.e., of maintaining the reaction temperature, is generally between about 1 and about 10 hours, preferably, between about 2 hours and about 6 hours, after which the reaction mixture is allowed to cool to ambient temperature and any unreacted sulfide is removed from the reacted mixture by filtration. If necessary, sufficient superatmospheric pressure is applied in order to maintain the reaction mixture in liquid phase under the other reaction conditions obtaining. The amount of superatmospheric pressure employed is not critical except that sufficient pressure is maintained in order to insure a liquid phase reaction mixture.

10 15 Many of the phosphites above mentioned are available commercially. For those specifically enumerated above which are not available commercially, it is a simple matter to effect a reaction between phosphorous trichloride or tribromide and the corresponding monohydric alcohol in 20 which the mole ratios of the alcohol to the phosphorous compound are maintained between 1:1 and about 3:1 depending upon whether or not it is desired to produce a mixture predominating in the mono-, di-, or tri-phosphite ester. Preferably a mole ratio of alcohol to phosphorous 25 trihalide of between about 0.75 and about 3.5 to 1 is maintained. Any solvents which are employed in effectuating the reaction are distilled off at atmospheric pressures or under slight vacuum, if need be.

One convenient method of producing an additive, although the following specific examples do not employ it, involves the use of lubricating oil fractions, middle distillate or residual fuel fractions as the reaction or solvent medium so that, upon a final filtration to remove any traces of unreacted sulfide, an oil concentration suitable 30 for direct addition to lubricating oils, middle distillate fuels or residual fuels may be accomplished without further treatment. Usually these oil-phospho-sulfurized phosphite ester concentrations will contain between about 50% and about 75% by weight of phospho-sulfurized 35 phosphite ester and may be marketed as such and they may be used in many instances as the direct and only additive for the materials in which they are to be ultimately employed.

40 The novel phospho-sulfurized phosphite esters are useful in lubricating oil compositions of the type employed in internal combustion engines of either the gasoline or diesel types as well as in heavy duty gas engine lubricants. The amounts incorporated into such lubricating oils range 45 between about 0.001 and about 10.0 wt. percent generally, preferably between about 0.01 and about 5.0 wt. percent. Additionally, the novel additives herein described 50 find usage in the middle distillate fuels and residual fuels for the purpose of imparting anti-rust and anti-corrosive properties to the fuels. Such fuels are those normally sold 55 commercially as gasoline, jet fuel, kerosene, heating oil fuel, and the heavy residual fuel oils such as Bunker-C. When so used, the additives are incorporated into these fuels in amounts ranging between about 0.001 and about 5.0 wt. percent, preferably between about 0.01 and about 60 1.5 wt. percent. All of the above percentage figures are based on the total weight of the composition.

65 The fuels and lubricating oil compositions described above may also include conventional additives present in like or smaller amounts, for example, they may contain oxidation inhibitors, such as phenyl alpha naphthylamine; rust inhibitors such as over-based alkaline earth metal petroleum sulfonates and alkyl amines; detergent additives such as over-based calcium petroleum sulfonate, phospho-sulfurized polyisobutylene, barium phenate sulfide, or a so-called ashless dispersant such as the polyisobutylene-substituted succinic anhydride reaction product with a polyethylene polyamine such as tetraethylene pentamine. Additionally, conventional additives particularly employed in lubricating oil compositions include 70 75 viscosity index improvers such as long chain wax alkyl-

ated naphthylene, the polymers of acrylates and methacrylates esterified with long chain monohydric alcohols, and the corresponding polymethacrylates.

Two typical specific lubricating motor oil bases have been employed. Both are of the SAE 10W-30 grade and they differ from one another only in a minor manner. In one case, the base oil is composed of 90.6% of a solvent extracted, dewaxed neutral oil from Mid-Continent paraffinic crude. It has a viscosity of 105-115 SUS (Saybolt Universal Seconds) at 100° F. and a pour point of about 0° F. The remaining 9.4% is the same type of oil but is one having a viscosity of about 450-500 SUS at 100° F. This oil base is employed in carrying out the Falex wear test. Another similar oil that is suitable as an oil base is composed of 90.75% of the same oil described before except that it has a viscosity of between about 150 and about 175 SUS at 100° F., the remainder of the oil base constituting the same oil as is used in the previously described blend in the amount of 9.4%. Both oils contain approximately 10.6% of a viscosity index improver, namely, polyisobutylene, and about 3.78% of an ashless dispersant identified as the polyisobutylene succinic anhydride imide of tetraethylene pentamine. The oil base comprised about 83% of the total compounded oil compositions plus minor amounts, i.e., less than 1%, of over-base calcium petroleum sulfonate and wax-alkylated naphthalene plus the copolymer of lorol fumarate with vinyl acetate. Where the novel antiwear and antioxidant additives are employed, they are used in the amount of 1.22 wt. percent, based on the total compounded composition.

The Falex wear test was made by running the test compositions in a Falex wear test machine. This test was conducted for the purpose of measuring the amount of wear which the bearings would encounter under extremely severe conditions using the test oil compositions. A steel pin is rotated at 290 r.p.m. between two V blocks for 30 minutes at 500 lbs. per square inch direct gauge pressure. The entire assembly is immersed in the test oil composition at ambient temperature. The wear performance of the test compounded oil is judged by the weight loss, in milligrams, of the steel pin. Pin seizure or borderline pin seizure conditions are avoided under the conditions, or, if they occur, the test oil is deemed to have failed in antiwear qualities.

A second test was carried out in order to evaluate the sludge-handling ability of the tested lubricating oil compositions in which the temperature of the oil was cyclically raised and lowered over a period of many hours in order to determine the oxidation stability and the sludge inhibiting or sludge forming tendencies of the novel additives in the oil compositions. A 6-cylinder Ford engine was used which employed a standard carburetor. It was operated at a standard speed of 1,500 r.p.m. plus or minus 15 r.p.m. under a constant load of 140 plus or minus 2 foot lbs. of torque. The oil sump temperature was maintained in the cold phase at 150° F. ±5° F. and at 215° F. ±5° F. in the hot phase. The cold phase operation was for a period of 5 hours and alternated with a hot phase operation of 2 hours. This is known as the Ford cyclic temperature sludge test.

Still another test was carried out known as a lubricant stability test which evaluates the compounded oils under accelerated oxidative conditions. The method is designed primarily to evaluate the stability of railroad Diesel lubricants wherein the compounded oils are subjected to elevated temperatures (342° F.) for a period of 23 hours in contact with copper-lead alloy, and silver, bearing metals, i.e., those encountered in heavy duty Diesel engines. Air is bubbled through the test oil while stirring it under these conditions and for the length of time indicated. Air is bubbled in at about 2 cubic feet per hour and the stirrer is rotated at about 600 r.p.m. Fresh metal specimens are inserted into the oil every three hours. Saybolt viscosities at 100° F. are measured and the rating

of the oil is computed on the basis of percent viscosity increase after 23 hours.

The invention will be more completely understood by reference to the following examples but it is to be distinctly understood that it is not to be limited to these examples since they are only exemplary or representative in nature. All percentages are with respect to weight percent.

#### EXAMPLE 1

10 25 grams of phosphorus pentasulfide was gradually added to 84 grams of triethyl phosphite over a period of about 1 hour. The reacting mixture was stirred for an additional 3 hours without the addition of externally supplied heat; at the end of which time the reaction mixture was clear and the reaction had stopped. The product analyzed 19.8 wt. percent of phosphorus and 16.3 wt. percent of sulfur.

#### EXAMPLE 2

20 About 279 grams of lorol alcohol was reacted with about 69 grams of phosphorous trichloride by gradually adding the same to the phosphorous trichloride at a temperature of about 10° C. over a period of two hours. Stirring was continued at room temperature until no more 25 gas was evolved. The reaction was completed after about 20 hours. The triester had a phosphorus content of 4.46 wt. percent.

25 About 120 grams of the trilorol phosphite was gradually admixed with about 20 grams of phosphorus pentasulfide at a temperature of about 90° C. over a period of about 6 hours. The reacted mixture was filtered to remove all unreacted phosphorus pentasulfide. The final product analyzed 6.04 wt. percent phosphorus and 7.60 wt. percent sulfur.

#### EXAMPLE 3

30 An SAE 10W-30 grade internal combustion engine lubricating oil was prepared. It contained about 75.29 wt. percent of a solvent extracted, de-waxed, neutral oil from Mid-Continent paraffinic crude having a viscosity of 105-115 SUS (Saybolt Universal Seconds) at 100° F. and a pour point of about 0° F.; about 7.7 wt. percent of the same type of oil but having a viscosity of about 450-500 SUS at 100° F.; about 10.5 wt. percent of a viscosity index improver (polyisobutylene); about 0.5 wt. percent of a pour point depressant (a wax alkylated naphthalene); about 3.75 wt. percent of an ashless dispersant (the condensation product of polyisobutylene succinic anhydride with tetraethylene pentamine); and slightly less than 1% of an ash forming detergent, i.e., an over-based calcium alkaryl sulfonate. In addition, in each of the tests, the base oil contained, as an additive, an antiwear agent in the amount of 1.22 wt. percent.

35 The compounded compositions were subjected to a standard Falex antiwear machine test for 30 minutes using a bearing pressure of 500 lbs. per square inch. The figures given in the following table show the weight loss of the steel pin, in milligrams.

#### TABLE

Bearing weight loss, milligrams

|                                                        |     |
|--------------------------------------------------------|-----|
| A—Base oil+phospho-sulfurized product of Example 1     | 3.3 |
| B—Base oil+phospho-sulfurized product of Example 2     | 3.6 |
| C—Base oil+conventional antiwear additive <sup>1</sup> | 7.4 |

<sup>1</sup> Zinc di-(C<sub>4</sub>-C<sub>6</sub> alkyl) dithiophosphate.

70 It is apparent from a consideration of the above data that the bearing weight loss in the case of the use of phospho-sulfurized phosphites as additives is only 50% of that attained in the use of a conventional antiwear additive and that automotive engine lubricating oils containing the phospho-sulfurized phosphites possess high qualities from the standpoint of antiwear properties.

7  
EXAMPLE 4

It was found that the use of the cyclic temperature sludging tests showed a definite inhibition of oxidation and a satisfactory dispersion of what little sludge was formed in the use of these phospho-sulfurized phosphites as compared with the same base oil without the phospho-sulfurized phosphites. The base oil, in all tests, was the same as that described in Example 3.

|                                                                              | Hours <sup>1</sup> |       |
|------------------------------------------------------------------------------|--------------------|-------|
|                                                                              | 105                | 126   |
| A—Base oil plus phospho-sulfurized product of Example 2 (1 wt. percent)----- | 9.07               | 5.8   |
| B—Base oil (no phospho-sulfurized additive)-----                             | 5.8                | ----- |

<sup>1</sup> Merit ratings: 10.0, no sludge; 0, most possible sludging.

## EXAMPLE 5

A further comparative series of lube oil oxidative stability tests were undertaken following the procedure hereinbefore set forth in order to determine the relative resistance to oxidation of the novel compounded lubricating oil. Oil A, the base oil, contained no phospho-sulfurized product but comprised about 90% of solvent dewaxed, neutral Mid-Continent lube oil having a viscosity of about 150 SUS at 100° F. and about 10% of polyisobutylene of 14,000–15,000 viscosity average molecular weight (Staudinger). Oil B was the same as Oil A but contained, in addition, about 1% of the phospho-sulfurized phosphite of Example 2.

## Lube stability test

|             | Percent viscosity increase<br>after 23 hours |
|-------------|----------------------------------------------|
| Oil A ----- | 100.0                                        |
| Oil B ----- | 8.3                                          |

Since this test measures the oxidative stability of the oil blends and the less the increase in viscosity the better the oil, it is readily apparent that the use of 1.0% of the product of Example 2 (Oil B) gives rise to a compounded oil of astonishing stability to oxidation.

Having now thus fully described and illustrated the nature of the invention, what is desired to be secured by Letters Patent is:

1. A hydrocarbon composition comprising a major amount of a hydrocarbon liquid selected from the group consisting of lubricating oils, middle distillate fuels, and residual fuels and between about 0.001 and about 10.0 wt. percent of the reaction product of organic phosphite esters having the formula:



wherein R<sub>1</sub> is a radical selected from the group consisting of alkyl, chloralkyl, aryl, chloraryl, aralkyl, chloraralkyl, cycloalkyl, chlorcycloalkyl, alkaryl, chloralkaryl, and R<sub>2</sub> and R<sub>3</sub> are hydrogen or the same as R<sub>1</sub>, with a polysulfide of phosphorus.

2. A hydrocarbon composition comprising a major amount of a hydrocarbon liquid selected from the group consisting of lubricating oils, middle distillate fuels, and residual fuels and between about 0.001 and about 10.0

wt. percent of the reaction product as in claim 1 wherein the phosphite ester is a triester.

3. A hydrocarbon composition comprising a major amount of a hydrocarbon liquid selected from the group consisting of lubricating oils, middle distillate fuels, and residual fuels and between about 0.001 and about 10.0 wt. percent of the reaction product as in claim 2 wherein the phosphite ester is a trialkyl phosphite ester.

4. A hydrocarbon composition comprising a major amount of hydrocarbon liquid selected from the group consisting of lubricating oils, middle distillate fuels, and residual fuels and between about 0.001 and about 10.0 wt. percent of the reaction product as in claim 3 wherein the trialkyl phosphite ester is trilrolol phosphite ester.

5. A hydrocarbon composition comprising a major amount of a hydrocarbon liquid selected from the group consisting of lubricating oils, middle distillate fuels, and residual fuels and between about 0.001 and about 10.0 wt. percent of the reaction product as in claim 3 wherein the trialkyl phosphite ester is triethyl phosphite.

6. A hydrocarbon composition comprising a major amount of a hydrocarbon liquid selected from the group consisting of lubricating oils, middle distillate fuels, and residual fuels and between about 0.001 and about 10.0 wt. percent of the reaction product as in claim 1 wherein the phosphorus polysulfide is phosphorus pentasulfide.

7. A hydrocarbon composition comprising a major amount of a hydrocarbon liquid selected from the group consisting of lubricating oils, middle distillate fuels, and residual fuels and between about 0.001 and about 10.0 wt. percent of the reaction product as in claim 3 wherein the phosphorus polysulfide is phosphorus pentasulfide.

8. A hydrocarbon composition comprising a major amount of a hydrocarbon lubricating oil and between about 0.001 and about 10.0 wt. percent of the reaction product as in claim 4.

9. A hydrocarbon composition comprising a major amount of a hydrocarbon lubricating oil and between about 0.001 and about 10 wt. percent of the reaction product as in claim 5.

10. A hydrocarbon composition comprising a major amount of a hydrocarbon lubricating oil and between about 0.001 and about 10 wt. percent of the reaction product as in claim 6.

11. A hydrocarbon composition comprising a major amount of a hydrocarbon lubricating oil and between about 0.001 and about 10 wt. percent of the reaction product as in claim 7.

50

## References Cited

## UNITED STATES PATENTS

|           |        |              |       |            |
|-----------|--------|--------------|-------|------------|
| 2,231,301 | 2/1941 | Smith        | ----- | 252—46.6   |
| 2,589,326 | 3/1952 | Oberright    | ----- | 252—46.6   |
| 2,595,170 | 4/1952 | Rudel et al. | ----- | 252—46.6   |
| 2,733,235 | 1/1956 | Cross et al. | ----- | 252—46.6 X |

DANIEL E. WYMAN, Primary Examiner

W. CANNON, Assistant Examiner

60

## U.S. CL. X.R.

44—76; 252—46; 260—921